

## UNITED STATES PATENT OFFICE

2,663,637

## PROCESS OF PRODUCING INTEGRAL COLOR CORRECTION MASKS

Karl Otto Ganguin and Norman Hulton Haddock,  
Blackley, Manchester, England, assignors to  
Imperial Chemical Industries Limited, a corpora-  
tion of Great Britain

No Drawing. Application August 1, 1949,  
Serial No. 108,045

Claims priority, application Great Britain  
August 20, 1948

6 Claims. (Cl. 95—2)

1

This invention relates to colouring processes and more particularly to colouring processes for use in colour photography.

The dyestuffs and pigments used in practice in subtractive processes of colour photography do not possess ideal special absorption curves. In addition to absorbing light in the desired part of the spectrum they also absorb some light in other parts of the spectrum and in consequence the colour reproduction obtained is never ideal. For example magenta dyestuffs formed by colour development absorb the desired complementary coloured green light and in addition always absorb undesirably a certain amount of blue light. It has been proposed (see for example The Journal of the Photographic Society of America, volume 13, 94-96, February 1947) to correct for these deficiencies by the use of an automatic masking method whereby coloured colour formers are used, the light absorption of the coloured colour former being equal or approximately equal to the undesired light absorption of the developed dyestuff. For example the colour former which is used in a photographic layer to form a magenta dyestuff on colour development may itself be coloured yellow so that it absorbs blue light at an intensity equal to the undesired blue absorption of the magenta dyestuff formed by colour development. Accordingly the unchanged colour former itself forms the coloured mask and the blue absorption of the photographic layer is a constant value (irrespective of the green absorption of the magenta image) which can be compensated for by using a suitable filter when printing.

The coloured colour formers it has been proposed to use in the above process are compounds containing the group  $-\text{N}=\text{N}-\text{R}$  where  $\text{R}$  is an aromatic or heterocyclic radical. The



group is split off during the development with an aromatic amino compound and replaced by the phenylimino radical derived from the aromatic amino compound. Apart from the difficulties caused by the use of a coloured layer, particularly in multi-layer films, the main practical objection to the above automatic masking process lies in the fact that the reaction of coloured colour formers of this kind with the aromatic amino compounds used for development is usually much slower than the reaction of the normal colourless colour formers with the aromatic amino compounds.

We have now discovered a new masking process

2

in which we obviate the practical difficulties involved in using this kind of coloured colour former. In our new masking process we use colourless colour formers, the yellow colour former being of a particular kind, and after developing the image with a colour forming developer, we treat the film with a gelatine hardening agent so that the residual colour former in selected parts of the film is rendered incapable of coupling with a diazonium compound, and subsequently we treat the film with a diazonium compound so that the residual colour former, which is still capable of coupling, is converted into the desired colour masks.

15 According to our invention we provide an improved process for colour photography which comprises developing with a colour forming developer, an exposed multilayer film wherein there is present in at least one of the layers, a yellow colour former which contains in its molecular structure the grouping  $-\text{CO}-\text{CH}_2\text{CO}-$  as part of an open chain of atoms, treating the film with a gelatine hardening agent, and subsequently treating the film with a solution of a diazonium compound.

20 The process of our invention is particularly valuable for use in three colour subtractive processes of colour photography in which there are used multilayer films which contain yellow, magenta and cyan colour formers in three separate layers, and in which the colours are formed by developing the films with alkaline solutions of aromatic amino compounds, such as for example p-diethylaminoaniline. In such processes to improve the fidelity of colour reproduction, a colour mask is required in the "magenta layer," (that is the layer containing the magenta colour former) to correct for the imperfect colour absorption of the magenta dyestuff, and to a smaller extent in the "cyan layer," to correct for the

25 imperfect colour absorption of the cyan dyestuff, but no mask is usually required in the "yellow layer." In the process of our invention the film after colour development contains residual colour former which is capable of reacting with a diazonium compound to form a colour mask but after treating the film with a gelatine hardening agent, the yellow colour formers of the kind hereinbefore defined, present in the "yellow layer" of the film, are unable to react with the diazonium compound and accordingly no mask is formed in the "yellow layer." This effect is a general effect obtained with different kinds of gelatine hardening agents. This effect is not completely understood but it appears to be associated with the

overall hardening of the "yellow layer" containing the specified colour former.

As examples of yellow colour formers suitable for use in the process of the present invention, there may be mentioned p-stearoylaminopenzoyl-acetanilide-p'-carboxylic acid, p-methoxybenzoylaceto-(2-N-octadecyl-N-methylamino)-5-carboxyanilide, p-stearoylaminobenzoylacetanilide-3:5-dicarboxylic acid.

The quantities of colour formers originally introduced into the "magenta layer" and the "cyan layer" may, if desired, be so adjusted that after exposure and colour development there is very little or no residual colour former in these layers in the areas of maximum exposure so that little or no colouring matter is formed in these areas of maximum exposure on treating the film with a solution of a diazonium compound and accordingly the overall fog of the masking image is reduced to a minimum. This forms a further feature of our invention. When the quantities of colour former are so adjusted, the treatment of the film with a hardening agent may be carried out before, during or after the bleaching of the silver, and any gelatine hardening agents, for example compounds of aluminum or chromium, can be used. For example there may be used potassium alum or chrome alum or there may be used the hardening agents used for the imagewise tanning of gelatine in the so-called "Carbon," "Carbro," "Collotype," "Bromoil" or "Transfer" processes (see for example "History of Color Photography" by J. S. Friedman, 1947, published by The American Photographic Publishing Company, Boston).

Alternatively the fog of the masking image can be controlled by carrying out the hardening treatment simultaneously with the bleaching out of the silver, that is to say by treating the film after exposure and colour development with a tanning-bleaching bath. This forms a still further feature of our invention. Examples of such tanning-bleaching baths are for example described in "History of Color Photography" by J. S. Friedman, 1947, pages 466, 467 and 468.

In this modification of the process all the residual yellow colour former is rendered incapable of coupling but seemingly in the "magenta layer" and "cyan layer" only imagewise hardening occurs since on treating the film with a solution of the diazonium compound coupling occurs counter-imagewise in these layers. In this modification of the process therefore it is unnecessary to adjust the quantity of colour formers incorporated in the emulsions in order to ensure that the colour former is substantially used up in the areas of maximum exposure.

The density and gradation of the masking images formed in the process can be controlled by adjusting the concentration and temperature of the solution of diazonium compound used in the process. The relative density and gradation of the masking images in the "magenta layer" and the "cyan layer" can be controlled by adjusting the relative concentration and nature of the colour formers used in the two layers. Alternatively the relative densities and gradation of the two masking images can be controlled by using as colour former in the "cyan layer" a mixture of a colour former of the 1-naphthol series with the 4-position unsubstituted, and a colour former of the 1-naphthol series with a substituent in the 4-position. This substituent in the 4-position prevents coupling with a diazonium compound but does not prevent reaction with the aromatic amino com-

5 pound used as colour-forming developer and this forms still a further feature of our invention. For example there may be used a mixture of the p-(methyl-octadecyl-amino)-anilide of 1-hydroxy-2-naphthoic acid and of the corresponding 4-sulphonic acid. The unsulphonated colour former will react either with the colour forming developer or with the diazonium compound but the sulphonated colour former will react only with the colour forming developer and not with the diazonium compound.

10 The diazonium compounds chosen for use in the formation of the masking images should be such as will react with the residual colour formers to give azo dyestuffs having the light absorption properties required to compensate, as far as possible, for the undesirable light absorption of the dyestuffs formed by the normal colour development with aromatic amino compounds. The solutions of the diazonium compounds may be prepared by diazotising the parent bases or alternatively they may be prepared from any available form of stabilised or passive diazonium compound (see for example "The Aromatic Diazo Compounds" by K. H. Saunders published by Edward Arnold & Co., London, 1936).

15 The process of our invention may be used to obtain positive masking images alongside the normal negative images obtained by simple exposure and colour development or alternatively it may be used in association with reversal processes so that negative masking images are obtained alongside the normal positive images and this forms a still further feature of our invention. For example the multilayer film may be first exposed to the light from an object or to the light transmitted by a colour transparency, developed with a black and white developer, the developed silver re-bleached to silver chloride and the latter dissolved out with, for example, sodium sulphite solution which does not affect the residual silver bromide. The film may then be fully exposed to light and subsequently processed by developing with a colour forming developer, bleach-tanning, treating with a diazonium compound and fixing. Alternatively if the quantities of colour formers in the "magenta layer" and "cyan layer" have been suitably adjusted, the film may be exposed to the image or to the light transmitted by a colour transparency, developed with a black and white developer, re-exposed and developed with a colour forming developer, tanned, treated with a diazonium compound, bleached and fixed.

20 25 30 35 40 45 50 55 60 65 70 75 The invention is illustrated but not limited by the following examples in which the parts are by weight.

#### EXAMPLE 1

A multilayer light sensitive photographic film is made up as follows:

A support material is coated with a layer of red light sensitised emulsion containing 10 grams per litre of the cyan image producing colour coupler described in Example 10 of British specification No. 465,823. Upon this layer there is coated a green light sensitised emulsion containing 10 grams per litre of the magenta image producing colour coupler described in Example 3 of British specification No. 502,663. A layer of colloidal silver is now coated on to act as a filter layer, and finally a layer of unsensitised emulsion containing 10 grams per litre of the sodium salt of p-stearyl-aminobenzoyl acetanilide-p'-carboxylic acid. The film is exposed to

5

light and developed in the developer made up by the following recipe.

|                                     |       |      |
|-------------------------------------|-------|------|
| p-diethylaminoaniline hydrochloride | grams | 3    |
| Sodium sulphite anhydrous           | do    | 1    |
| Sodium carbonate                    | do    | 60   |
| Potassium bromide                   | do    | 2    |
| Water                               | cc    | 1000 |

The film is rinsed and transferred into a tanning-bleaching bath made up by mixing equal parts of the following Solutions A and B.

*Solution A*

|                        |       |      |
|------------------------|-------|------|
| Potassium ferricyanide | Parts | 15   |
| Potassium bromide      | 37.5  |      |
| Potassium dichromate   | 36.25 |      |
| Acetic acid            | 37.5  |      |
| Water to               | 10.0  |      |
|                        |       | 1000 |

*Solution B*

|                |       |      |
|----------------|-------|------|
| Potassium alum | Parts | 50   |
| Water to       |       | 1000 |

The film is washed again, then treated with a 1% solution of the zinc chloride double salt of p-nitrobenzene diazonium chloride, washed and finally fixed with a 20% solution of sodium thiosulphate.

After this treatment the red sensitive layer contains a cyan dyestuff negative image and also a red azo dyestuff positive image which serves as a mask to correct for the undesirable absorption of blue and green light by the cyan dyestuff. The green sensitive layer contains a magenta dyestuff negative image and also a yellow azo dyestuff positive image, which serves as a mask to correct for the undesirable absorption of blue light by the magenta dyestuff.

The blue sensitive layer contains a yellow dyestuff negative image but no corresponding azo dyestuff positive image. When the negative film so obtained is used for making positive prints or "dupe" or separation negatives, much improved colour fidelity and saturation is obtained as compared with reproductions from negative colour film which contain the same negative dyestuff images made by colour development but no corresponding azo positive images.

**EXAMPLE 2**

A multilayer light sensitive photographic element is made up as follows:

A support material is coated with a layer of red light sensitised emulsion containing 2 grams per litre of the p-(methyl-octadecyl-amino)-anilide of 1-hydroxy-2-naphthoic acid and 8 grams per litre of the sodium salt of the corresponding 4-sulphonic derivative. The other layers are made up as in Example 1.

The material is exposed to light transmitted by a colour negative or positive transparency and developed in the developer made up by the following recipe:

|                           |       |      |
|---------------------------|-------|------|
| Sodium sulphite anhydrous | Grams | 25   |
| Metol                     | do    | 2    |
| Hydroquinone              | do    | 14   |
| Potassium bromide         | do    | 2    |
| Potassium thiocyanate     | do    | 2.5  |
| Sodium hydroxide          | do    | 2    |
| Potassium carbonate       | do    | 1000 |

6

|                           |      |
|---------------------------|------|
| Sodium sulphate anhydrous | 10   |
| Water                     | 1000 |

After washing, the film is transferred into a bleaching solution made up by the following recipe:

|                        |       |      |
|------------------------|-------|------|
| Potassium ferricyanide | grams | 100  |
| Sodium chloride        | do    | 50   |
| Water                  | cc    | 1000 |

10 The developed silver is thus bleached to silver chloride. The film is then treated with a 20% solution of sodium sulphite which dissolves the silver chloride, but leaves the residual silver bromide unaffected.

15 The material is now exposed to the light from a tungsten lamp, developed in the colour developer of Example 1 and then further processed as described in Example 1. Instead of the diazo compound used in Example 1, the diazonium

20 compounds derived from 4-nitro-6-methoxyaniline, 4-methoxy-6-nitroaniline, 4-aminodiphenylamine, 4-benzoylaminio-6-methoxyaniline or any other diazonium compounds which couple with colour formers to give the colours needed for masking purposes may be used.

25 The processed film contains in the red sensitive layer a cyan dyestuff positive image and a red dyestuff negative image, which serves as a mask to correct the too low transmission of blue and green light by the cyan dyestuff. The green sensitive layer contains a magenta dyestuff positive image and a yellow dyestuff negative image, which serves as a mask to correct for the absorption

30 of blue light by the magenta dyestuff.

35 The blue sensitive layer contains a yellow dyestuff positive image but no corresponding azo dyestuff negative image. The negative or positive "dupe" prints so obtained show improved colour fidelity and brightness compared with

40 "dupe" prints made without colour correction masks.

**EXAMPLE 3**

45 A multilayer light sensitive material is made up as follows:

46 A support material is coated with a layer of red light sensitive emulsion containing 6 grams per litre of the sulphonated condensation product described in Example 10 of British specification No. 465,823 and 2 grams per litre of the corresponding unsulphonated condensation product.

47 Upon this layer is coated a green light sensitised emulsion containing 4 grams per litre of the magenta image producing colour coupler described in Example 3 of British specification No. 502,665. A colloidal silver layer is now coated on to act as a yellow filter layer and as the top layer an unsensitised emulsion is coated containing 10 grams per litre of the sodium salt of p-stearyl - aminobenzoylacetylalide - p'-carboxylic acid.

48 The material is exposed to light and developed with the colour developer used in Example 1.

49 After washing, the film is treated with a hardening bath containing 2.5% potassium chrome alum. The film is washed again and transferred to a bleaching bath of the following composition:

|                        |       |      |
|------------------------|-------|------|
| Potassium ferricyanide | Grams | 50   |
| Potassium bromide      | do    | 20   |
| Water                  | cc    | 1000 |

50 The film is washed and soaked in a 1% solution of the zinc chloride double salt of 2-meth-

oxy-4-nitrobenzene diazonium chloride. It is not necessary in the process of this example to use an imagewise tanning-bleaching bath since the amounts of colour former incorporated in the green and red sensitive layers are so adjusted that no residual colour former is left in the areas of maximum exposure. The reaction between the colour former of the blue sensitive layer and the diazonium compound is prevented by the treatment of the film in the hardening bath. After final fixing the colour negative obtained shows improvements similar to those of the negative obtained in Example 1.

## EXAMPLE 4

A multilayer film is made up as described in Example 3.

After exposure to light the film is developed with the black and white developer used in Example 2, and after washing and re-exposure it is developed in the colour forming developer used in Example 1. Then the material is hardened in the hardening solution made up according to the following recipe:

|                      |       |      |
|----------------------|-------|------|
| Potassium alum       | grams | 30   |
| Sodium acetate       | do    | 60   |
| Water                | cc.   | 1000 |
| Acetic acid, glacial | cc.   | 5    |

The film is transferred into a 1% solution of the zinc chloride double salt of 2-methoxy-4-nitrobenzene diazonium chloride. It is then bleached, fixed and finally washed.

The transparency obtained is of the reversal type and has features and improvements similar to those of the transparency obtained in Example 2.

## EXAMPLE 5

A multilayer light sensitive material is made up as follows:

A support material is coated with a layer of red light sensitized emulsion containing 10 grams per litre of the sodium salt of 1-hydroxy-4-sulphonaphthoyl (2)-octadecylamide. Upon this layer is coated a green light sensitized emulsion containing 10 grams per litre of the 1:3-bis-( $\beta$ -cyanoacetyl)-5-octadecylamino benzene. A colloidal silver layer is now coated on and as the top layer an unsensitised emulsion is coated containing 10 grams per litre of the sodium salt of p-stearylaminobenzoylacetanilide-p'-carboxylic acid. The material is exposed to light and developed with the colour developer used in Example 1. The film is washed and then treated with the hardening solution used in Example 4. The film is washed and then transferred to the bleaching bath used in Example 4.

The material is again washed and then immersed in a 0.5% solution of the zinc chloride double salt of 2-nitro-4-methoxy-benzene diazonium chloride, and finally fixed and washed. The colour negative obtained carries a cyan negative image in the layer next to the support, a magenta negative image and a yellow azo dyestuff positive masking image in the next layer, a clear gelatin layer left after bleaching of the colloidal silver, and finally a yellow negative image in the upper layer.

We claim:

1. A process for the production of subtractively colored photographic transparencies with color correction masks from multi-layer film having differently sensitized silver halide emulsion layers containing color formers adapted to form yellow,

magenta, and cyan images in separate layers by coupling with the development product of a primary aromatic amino developing agent and being capable of producing azo dyes by coupling with a diazonium compound, wherein the color former which is adapted to form a yellow image contains in its molecular structure the group  $-\text{CO}-\text{CH}_2\text{CO}-$  as part of an open chain of atoms, which comprises exposing the film to light, color developing to said color images by treating said layers with said primary aromatic amino developing agent, treating the film with a gelatin hardening agent selected from the group consisting of chromium and aluminum gelatin hardening compounds to render the residual color former in the yellow image layer incapable of coupling with a diazonium compound, subsequently treating the film with a solution of a diazonium compound to convert residual color former in the magenta and cyan colored layers into masking images and retaining the color images and masking images in said layers.

2. A process for the production of subtractively colored photographic transparencies as set forth in claim 1 wherein said color former containing in its molecular structure the group



as part of an open chain of atoms is selected from the group consisting of p-stearoyl-aminobenzoyl-acetanilide-p'-carboxylic acid, p-methoxy-benzoylaceto-(2-N-octadecyl-N-methylamino)-5-carboxyanilide, and p-stearylaminobenzoylacetanilide-3:5-dicarboxylic acid.

3. A process for the production of subtractively colored photographic transparencies as set forth in claim 1 wherein the quantities of magenta and cyan color formers in said differently sensitized silver halide emulsion layers are so adjusted that after exposure and color development there is substantially no residual magenta or cyan color former in the areas of maximum exposure of their respective layers.

4. A process for the production of subtractively colored photographic transparencies as set forth in claim 1 wherein the treatment with the gelatin hardening agent is carried out simultaneously with the bleaching out of the developed silver.

5. A process for the production of subtractively colored photographic transparencies as set forth in claim 1 wherein the cyan color former is a mixture of a color former of the 1-naphthol series with the 4-position unsubstituted and a color former of the 1-naphthol series with a substituent in the 4-position.

6. A process for the production of subtractively colored photographic transparencies as set forth in claim 1 wherein prior to color developing to said color images, the multi-layer film is first exposed to light, developed with a black and white developer, bleached, and then fully exposed to light.

KARL OTTO GANGUIN.  
NORMAN HULTON HADDOCK.

## References Cited in the file of this patent

## UNITED STATES PATENTS

| 70 | Number    | Name         | Date           |
|----|-----------|--------------|----------------|
|    | 2,297,732 | Woodward     | Oct. 6, 1942   |
|    | 2,306,410 | Schinzel     | Dec. 29, 1942  |
|    | 2,431,996 | Duerr et al. | Dec. 2, 1947   |
|    | 2,449,966 | Hanson       | Sept. 21, 1948 |
| 75 | 2,518,739 | Young        | Aug. 15, 1950  |